



US005599474A

**United States Patent**

[19]

**Weiss et al.**[11] **Patent Number:** **5,599,474**[45] **Date of Patent:** **Feb. 4, 1997**[54] **TEMPERATURE INDEPENDENT  
MAGNETORHEOLOGICAL MATERIALS**[75] Inventors: **Keith D. Weiss; J. David Carlson,**  
both of Cary; **Theodore G. Duclos,**  
**Holly Springs; Kirk J. Abbey,** Raleigh,  
all of N.C.[73] Assignee: **Lord Corporation,** Cary, N.C.[21] Appl. No.: **229,270**[22] Filed: **Apr. 18, 1994****Related U.S. Application Data**[63] Continuation-in-part of Ser. No. 968,735, Oct. 30, 1992,  
abandoned.[51] **Int. Cl.<sup>6</sup>** ..... **H01F 1/44**[52] **U.S. Cl.** ..... **252/62.52; 252/62.54;**  
**252/62.56**[58] **Field of Search** ..... **252/62.52, 62.54,**  
**252/62.56, 74, 75**[56] **References Cited****U.S. PATENT DOCUMENTS**

|            |         |                  |           |
|------------|---------|------------------|-----------|
| Re. 32,573 | 1/1988  | Furumura et al.  | 252/62.52 |
| 2,575,360  | 11/1951 | Rabinow          | .         |
| 2,661,596  | 12/1953 | Winslow          | .         |
| 2,661,825  | 12/1953 | Winslow          | .         |
| 2,663,809  | 12/1953 | Winslow          | .         |
| 2,667,237  | 1/1954  | Rabinow          | .         |
| 2,670,749  | 3/1954  | Gemer            | .         |
| 2,733,792  | 2/1956  | Saxl             | .         |
| 2,751,352  | 6/1956  | Bondi            | 252/62.52 |
| 2,847,101  | 8/1958  | Bergmann         | 252/62.52 |
| 2,886,151  | 5/1959  | Winslow          | .         |
| 3,010,471  | 11/1961 | Gross            | .         |
| 3,700,595  | 10/1972 | Kaiser           | 252/62.52 |
| 3,764,540  | 10/1973 | Khalfalla et al. | 252/62.52 |
| 3,917,538  | 11/1975 | Rosensweig       | 252/62.52 |

|           |         |                 |           |
|-----------|---------|-----------------|-----------|
| 4,356,098 | 10/1982 | Chagnon         | 252/62.51 |
| 4,824,587 | 4/1989  | Kwon et al.     | 252/62.54 |
| 4,976,883 | 12/1990 | Kanno et al.    | 252/62.52 |
| 4,992,190 | 2/1991  | Shtarkman       | 252/62.52 |
| 5,007,513 | 4/1991  | Carlson         | 252/62.52 |
| 5,013,471 | 5/1991  | Ogawa           | 252/62.52 |
| 5,143,637 | 9/1992  | Yokouchi et al. | 252/62.52 |
| 5,147,573 | 9/1992  | Chagnon         | 252/61.51 |
| 5,167,850 | 12/1992 | Shtarkman       | 252/62.52 |
| 5,382,373 | 1/1995  | Carlson et al.  | 252/62.55 |

**FOREIGN PATENT DOCUMENTS**

|           |         |                    |
|-----------|---------|--------------------|
| 162371    | 10/1952 | Australia          |
| 406692    | 1/1991  | European Pat. Off. |
| 63-175401 | 7/1988  | Japan              |

**OTHER PUBLICATIONS**

*Technical News Bulletin*, vol. 32, No. 5, pp. 54-60, U.S. Dept. of Commerce (May 1948) (describes magnetic clutch developed at National Bureau of Standards by J. Rabinow). *Kirk-Othmer Encyclopedia of Chemical Technology*, vol. 14, pp. 662-664 (1981) (Month Unknown).

Primary Examiner—Prince Willis, Jr.

Assistant Examiner—Alan D. Diamond

Attorney, Agent, or Firm—Wayne W. Rupert

[57] **ABSTRACT**

A magnetorheological material containing a particle component and a carrier fluid or mixture of carrier fluids having a change in viscosity per degree temperature ( $\Delta\eta/\Delta T$  ratio) less than or equal to about 16.0 centipoise/ $^{\circ}\text{C}$ . over the temperature range of about 25 $^{\circ}\text{C}$ . to -40 $^{\circ}\text{C}$ . The magnetorheological material exhibits a substantial magnetorheological effect and excellent lubricating properties with a minimal variation in mechanical properties with respect to changes in temperature. The magnetorheological material is advantageous in that it provides for the design of devices that are smaller, more efficient and consume less power.

**26 Claims, 4 Drawing Sheets**



Figure 1



Figure 2



Figure 3



Figure 4

## TEMPERATURE INDEPENDENT MAGNETORHEOLOGICAL MATERIALS

This is a continuation-in-part of application Ser. No. 07/968,735 filed on Oct. 30, 1992 now abandoned.

### FIELD OF THE INVENTION

The present invention relates to certain fluid materials which exhibit substantial increases in flow resistance when exposed to magnetic fields. More specifically, the present invention relates to low viscosity magnetorheological materials that substantially minimize the variance in force required by a magnetorheological device over a given temperature range.

### BACKGROUND OF THE INVENTION

Fluid compositions which undergo a change in apparent viscosity in the presence of a magnetic field are commonly referred to as Bingham magnetic fluids or magnetorheological materials. Magnetorheological materials normally are comprised of ferromagnetic or paramagnetic particles, typically greater than 0.1 micrometers in diameter, dispersed within a carrier fluid and in the presence of a magnetic field, the particles become polarized and are thereby organized into chains of particles within the fluid. The chains of particles act to increase the apparent viscosity or flow resistance of the overall material and in the absence of a magnetic field, the particles return to an unorganized or free state and the apparent viscosity or flow resistance of the overall material is correspondingly reduced. These Bingham magnetic fluid compositions exhibit controllable behavior similar to that commonly observed for electrorheological materials, which are responsive to an electric field instead of a magnetic field.

Both electrorheological and magnetorheological materials are useful in providing varying damping forces within devices, such as dampers, shock absorbers and elastomeric mounts, as well as in controlling torque and or pressure levels in various clutch, brake and valve devices. Magnetorheological materials inherently offer several advantages over electrorheological materials in these applications. Magnetorheological fluids exhibit higher yield strengths than electrorheological materials and are, therefore, capable of generating greater damping forces. Furthermore, magnetorheological materials are activated by magnetic fields which are easily produced by simple, low voltage electromagnetic coils as compared to the expensive high voltage power supplies required to effectively operate electrorheological materials. A more specific description of the type of devices in which magnetorheological materials can be effectively utilized is provided in U.S. Pat. Nos. 5,284,330 and 5,277,281.

Magnetorheological or Bingham magnetec fluids are distinguishable from colloidal magnetic fluids or ferrofluids. In colloidal magnetic fluids the particles are typically 0.005 to 0.01 micrometers in diameter. Upon the application of a magnetic field, a colloidal ferrofluid does not exhibit particle structuring or the development of a resistance to flow. Instead, colloidal magnetic fluids-experience a body force on the entire material that is proportional to the magnetic field gradient. This force causes the entire colloidal ferrofluid to be attracted to regions of high magnetic field strength.

Magnetorheological fluids and corresponding devices have been discussed in various patents and publications. For example, U.S. Pat. No. 2,575,360 provides a description of

an electromechanically controllable torque-applying device that uses a magnetorheological material to provide a drive connection between two independently rotating components, such as those found in clutches and brakes. A fluid composition satisfactory for this application is stated to consist of 50% by volume of a soft iron dust, commonly referred to as "carbonyl iron powder", dispersed in a suitable liquid medium such as a light lubricating oil.

Another apparatus capable of controlling the slippage between moving parts through the use of magnetic or electric fields is disclosed in U.S. Pat. No. 2,661,825. The space between the moveable parts is filled with a field responsive medium. The development of a magnetic or electric field flux through this medium results in control of resulting slippage. A fluid responsive to the application of a magnetic field is described to contain carbonyl iron powder and light weight mineral oil (2-10 centipoise).

U.S. Pat. No. 2,886,151 describes force transmitting devices, such as clutches and brakes, that utilize a fluid film coupling responsive to either electric or magnetic fields. An example of a magnetic field responsive fluid is disclosed to contain reduced iron oxide powder and a lubricant grade oil having a viscosity of from 2 to 20 centipoises at 25° C.

The construction of valves useful for controlling the flow of magnetorheological fluids is described in U.S. Pat. Nos. 2,670,749 and 3,010,471. The magnetic fluids applicable for utilization in the disclosed valve designs include ferromagnetic, paramagnetic and diamagnetic materials. A specific magnetic fluid composition specified in U.S. Pat. No. 3,010,471 consists of a suspension of carbonyl iron in a light weight hydrocarbon oil. Magnetic fluid mixtures useful in U.S. Pat. No. 2,670,749 are described to consist of a carbonyl iron powder dispersed in either a silicone oil or a chlorinated or fluorinated suspension fluid.

Various magnetorheological material mixtures are disclosed in U.S. Pat. No. 2,667,237. The mixture is defined as a dispersion of small paramagnetic or ferromagnetic particles in either a liquid, coolant, antioxidant gas or a semi-solid grease. A preferred composition for a magnetorheological material consists of iron powder and light machine oil. A specifically preferred magnetic powder is stated to be carbonyl iron powder with an average particle size of 8 micrometers. Other possible carrier components include kerosene, grease, and silicone oil.

U.S. Pat. Nos. 4,992,190 and 5,167,850 disclose rheological materials that are responsive to a magnetic field. The composition of these materials are disclosed to be either magnetizable particles and silica gel or carbon fibers dispersed in a liquid carrier vehicle. The magnetizable particles can be powdered magnetite or carbonyl iron powders with insulated reduced carbonyl iron powder, such as that manufactured by GAF Corporation, being specifically preferred. The liquid-carrier vehicle is described as having a viscosity in the range of 1 to 1000 centipoises at 100° F. Specific examples of suitable vehicles include Conoco LVT oil, kerosene, light paraffin oil, mineral oil, and silicone oil. A preferred carrier vehicle is silicone oil having a viscosity in the range of about 10 to 1000 centipoise at 100° F.

U.S. Pat. No. 2,751,352 and Australian Patent Specification 162,371 discloses magnetorheological fluids wherein the magnetic particles are inhibited from precipitating or settling out of the fluid system. The inhibition of particle settling is accomplished by the addition of a minute amount of an oleophobic material to the magnetic fluid. Examples of these oleophobic materials include ethyl alcohol, propyl alcohol, glycerol, ethylene glycol, propylene glycol and

ethylene diamine. The base carrier or vehicle for the magnetic particles is stated to be selected from a wide variety of materials preferably oleaginous in character. Examples of the base carrier or vehicle include mineral oils (40 to 2,000 SUS at 100° F.); synthetic lubricants produced by the Fischer-Tropsch, Synthol, Synthine, Berguis, and Voltolization processes; organic synthetic lubricants; synthetic lubricants made by the polymerization of alkylene oxides at elevated temperatures in the presence of catalysts (i.e., iodine, hydrogen iodide, etc.); polymers obtained from oxygen-containing heterocyclic compounds; silicone compounds; and fluoro and/or chloro carbon oils. While most of the base carriers or vehicles are only described as general classes of materials, specific compounds listed as carrier vehicles include light machine oil having a viscosity between 300 to 700 SUS at 100° F., di(2-ethylhexyl) sebacate, di(2-ethylhexyl) adipate, ethyl ricinoleate, tricresyl phosphate, trioctyl phosphate, dibutyl trichloromethane-phosphonate, trixyl phosphate, tributyl phosphate, triethyl phosphate, tetraphenyl silicate, tetra ethyl hexyl silicate, kerosene, and hexachlorobutadiene.

It is desirable that the continuous component or carrier fluid of a magnetorheological material exhibit several basic characteristics. These characteristics include: (a) chemical compatibility with both the particle component of the fluid and device materials; (b) relatively low cost; (c) low thermal expansion; (d) high density and (e) excellent lubricity. Magnetorheological materials should also be non-hazardous to the surrounding environment and, more importantly, be capable of functioning consistently over a broad temperature range.

Most of the carrier fluid components that are traditionally used in magnetorheological materials as previously described cannot adequately meet all of these basic requirements. For instance, many of the previously described magnetorheological materials cause large variations in the force exhibited by a magnetorheological device utilizing the materials over a broad temperature range. In addition, many of these traditional magnetorheological materials provide inadequate lubricating properties between device components. Hence, many of the magnetorheological materials prepared with traditional carrier fluids limit either the useful life of a device through excessive wear or the temperature range over which the device can be used. Conventional magnetorheological materials cannot be effectively utilized in automotive and aerospace damping devices and the like which require consistent application of precisely controlled force over widely varying temperatures.

Characterization of the performance of magnetorheological materials with respect to a change in operating temperature is vital to the successful commercialization of most magnetorheological devices, such as clutches, brakes, dampers, shock absorbers and engine mounts. All of these devices inherently experience a variation in operating temperature over their lifetime. For instance, specifications for automotive and aerospace applications typically require the device to operate at or survive exposure to temperatures ranging from about -40° C. to 150° C.

A need therefore exists for magnetorheological materials that are lubricating in nature and exhibit limited variation in properties over a broad temperature range.

#### SUMMARY OF THE INVENTION

The present invention is a magnetorheological material which exhibits a substantial magnetorheological effect, excellent lubricity, and a minimal variation in mechanical

properties with respect to changes in temperature. More specifically, the present invention relates to a magnetorheological material comprising a carrier fluid and a particle component wherein the carrier fluid has a change in viscosity ( $\eta$ ) per degree temperature (T) ( $\Delta\eta/\Delta T$  ratio) less than or equal to about 16.0 centipoise/°C. over the temperature range of about 25° C. to -40° C.

It has presently been discovered that carrier fluids having a  $\Delta\eta/\Delta T$  ratio less than or equal to about 16.0 centipoise/°C. over the temperature range of 25° to -40° C. can be utilized to prepare magnetorheological materials which have an unusually low variance of mechanical properties over a broad temperature range. Conventional carrier fluids, typically, have either a  $\Delta\eta/\Delta T$  ratio greater than the limit described above or poor lubricating properties and are therefore unacceptable for utilization in a device over an extended period of time or a broad temperature range. Carrier fluids that exhibit the necessary  $\Delta\eta/\Delta T$  ratio and lubricating properties for purposes of the invention have presently been found to exist sporadically within several major classes or groups of lubricating oils, such as unsaturated hydrocarbon oils; monobasic acid esters; glycol esters and ethers, fluorinated esters and ethers; silicate esters; silicone oils; and halogenated hydrocarbons. Various mixtures of lubricating oils have also presently been discovered to exhibit the necessary  $\Delta\eta/\Delta T$  ratio and lubricating properties required by the present invention. Magnetorheological materials utilizing the carrier fluids of the present invention when utilized in a device, such as a damper, mount or clutch, exhibit excellent lubricating properties and significantly less variation in the force output over a temperature range from about -40° to 150° C. as compared to devices using magnetorheological materials prepared with traditional carrier fluids.

#### BRIEF DESCRIPTION OF THE DRAWINGS

FIGS. 1-4 show the force output for a linear magnetorheological damper plotted as a function of temperature. The force data obtained for this damper at a magnetic field of about 1000 Oersted is measured over the temperature range of -40° to 150° C.

In FIG. 1 the force data obtained using a low viscosity magnetorheological material of the present invention (Example 44) is contrasted against data obtained with this damper under similar conditions using a comparative magnetorheological material (Example 45).

In FIG. 2 the force data obtained using a low viscosity magnetorheological material of the present invention (Example 46) is contrasted against data obtained with this damper under similar conditions using a comparative magnetorheological material (Example 49).

In FIG. 3 the force data obtained using a low viscosity magnetorheological material of the present invention (Example 47) is contrasted against data obtained with this damper under similar conditions using a comparative magnetorheological material (Example 50).

In FIG. 4 the force data obtained using a low viscosity magnetorheological material of the present invention (Example 48) is contrasted against data obtained with this damper under similar conditions using a comparative magnetorheological material (Example 51).

#### DETAILED DESCRIPTION OF THE INVENTION

The magnetorheological material of the present invention comprises a carrier fluid and a particle component wherein

the carrier fluid has a change in viscosity per degree temperature  $\Delta\eta/\Delta T$  ratio over the temperature range of about 25° C. to -40° C. less than or equal to about 16.0 centipoise/°C., preferably less than or equal to about 9.0 centipoise/°C., with less than or equal to about 7.0 centipoise/°C. being especially preferred. As utilized herein, the term "appropriate  $\Delta\eta/\Delta T$  ratio" refers to a  $\Delta\eta/\Delta T$  ratio over the temperature range of about 25° C. to -40° C. that is less than or equal to about 16.0 centipoise/°C.

Carrier fluids having an appropriate  $\Delta\eta/\Delta T$  ratio for purposes of the present invention may be found to sporadically exist in any of the known classes of oils or liquids with the exception of (a) natural fatty oils, (b) mineral oils, (c) polyphenylethers, (d) dibasic acid esters, (e) neopen-  
10 tylopolyl esters, (f) phosphate esters, and (g) synthetic cycloparaffins and synthetic paraffins. The known liquids that are classified within these six broad classes of liquids either do not exhibit the necessary  $\Delta\eta/\Delta T$  ratio, as exemplified by groups (a) through (e) or do not exhibit the lubricating properties necessary to satisfactorily be utilized in a magnetorheological fluid device, such as a damper, operated over a broad temperature range, as exemplified by groups (f) and (g).

The classes of oils or liquids in which a carrier fluid having an appropriate  $\Delta\eta/\Delta T$  ratio for purposes of the present invention may be found to sporadically exist include (h) unsaturated hydrocarbon oils; (i) monobasic acid esters; (j) glycol esters and ethers, (k) fluorinated esters and ethers; (l) silicate esters; (m) silicone oils; and (n) halogenated hydrocarbons, as well as mixtures and derivatives thereof. A carrier fluid mixture appropriate to the present invention will always be obtained independent of the amounts of each fluid present in the mixture when each fluid independently exhibits an appropriate  $\Delta\eta/\Delta T$  ratio and is selected from the classes (h) through (n). The preferred carrier fluids or carrier fluid mixtures of the present invention are selected from the classes (h), (j), (k), and (m). Although a large number of carrier fluids are classified within each of these broad classes, only a very limited number of these carrier fluids will exhibit the appropriate  $\Delta\eta/\Delta T$  ratio and therefore are appropriate for use in the present invention. Carrier fluids having a  $\Delta\eta/\Delta T$  ratio suitable for use in the present invention and falling within the classes (h) through (n) above are hereinafter collectively referred to as Group I carrier fluids. It should be noted that all fluids falling within classes (h) through (n) have lubricating properties suitable for purposes of the present invention regardless of the value of their  $\Delta\eta/\Delta T$  ratios.

A limited number of carrier fluid mixtures having an appropriate  $\Delta\eta/\Delta T$  ratio and necessary lubricating properties may also be obtained by mixing specific amounts of Group I carrier fluids described above that exhibit the appropriate  $\Delta\eta/\Delta T$  ratio with carrier fluids from classes (a) through (n) that are outside the scope of present invention in that they do not exhibit an appropriate  $\Delta\eta/\Delta T$  ratio or do not possess adequate lubricating properties. Carrier fluids falling within the classes of (a) through (n) above that do not exhibit an appropriate  $\Delta\eta/\Delta T$  ratio or do not possess adequate lubricating properties for purposes of the invention are herein-after collectively referred to as Group II carrier fluids. This particular mixture is hereinafter described as a primary fluid mixture. The specific amounts of each fluid added to prepare this primary fluid mixture is dependent upon the magnitude of the individual  $\Delta\eta/\Delta T$  ratios and lubricating properties exhibited by each fluid. In general, a primary fluid mixture appropriate to the present invention is obtained when the Group I and Group II carrier fluids are combined in a Group  
55

I:Group II carrier fluid weight ratio of about 85:15, preferably about 75:25, with a weight ratio of about 50:50 being especially preferred. The preferred primary fluid mixtures of the present invention contain a Group I carrier fluid selected from the group consisting of the carrier fluid classes (h), (j), (k) and (m) mixed with a Group II carrier fluid selected from group consisting of the carrier fluid classes (a), (b), (d), (g), (h), (j), (k) or (m).

Although many of the carrier fluids selected from groups (f) and (g) exhibit acceptable  $\Delta\eta/\Delta T$  ratios, they lack the necessary lubricating properties required by the present invention to insure a long life-time for a magnetorheological fluid device. Thus a limited number of carrier fluid mixtures appropriate to the present invention can also be obtained by mixing specific amounts of fluids selected from groups (f) and (g) that exhibit acceptable  $\Delta\eta/\Delta T$  ratios with fluids selected from groups (a) through (e) and (h) through (n) that do not exhibit an appropriate  $\Delta\eta/\Delta T$  ratio for purposes of the present invention. This particular mixture is hereinafter described as a secondary fluid mixture and carrier fluids falling within the classes (f) and (g) and exhibiting an appropriate  $\Delta\eta/\Delta T$  ratio are hereinafter collectively referred to as Group III carrier fluids, while those carrier fluids falling within the classes (a) through (e) and (h) through (n) and not exhibiting an appropriate  $\Delta\eta/\Delta T$  ratio are hereinafter collectively referred to as Group IV carrier fluids. Due to molecular interactions between the different fluids that make up the secondary fluid mixture, it has been discovered that it is possible for this fluid mixture, provided the fluids are properly selected, to unexpectedly exhibit a  $\Delta\eta/\Delta T$  ratio that is less than the  $\Delta\eta/\Delta T$  ratios of the individual fluids used in the preparation of the mixture. In general, a secondary fluid mixture appropriate to the present invention is obtained when the Group III and Group IV carrier fluids are combined in a Group III:Group IV carrier fluid weight ratio of about 85:15, preferably about 75:25, with a weight ratio of about 50:50 being especially preferred. The preferred secondary fluid mixtures of the present invention contain a Group III carrier fluid from class (g) mixed with a Group IV carrier fluid selected from the group consisting of classes (a), (b), (d), (h), (j), or (k).

The silicone oils, class (m), of the invention can be any polysiloxane, such as a silicone homopolymer or copolymer, comprising a siloxane polymeric backbone substituted with hydrocarbon radicals as side and end groups. The hydrocarbon radicals can be either straight chain, branched or cyclic, as well as aliphatic or aromatic with the number of carbon atoms ranging from 1 to about 8. In addition, the hydrocarbon radicals may contain H, N, O, S, Cl, Br and F functionality as in the case of fluorinated polysiloxanes. Examples of commercially available polysiloxanes include polydimethylsiloxanes, polymethylphenylsiloxanes, poly(methyl3,3,3-trifluoropropyl) siloxanes, polychlorophenyl-methylsiloxanes, dimethyl(tetrachlorophenyl)siloxane copolymers, dimethyl(phenylmethyl)siloxane copolymers, dimethyl(diphenyl)siloxane copolymers, and methyl3,3,3-trifluoropropyl(dimethyl)siloxane copolymers with polydimethylsiloxanes being preferred. In order for the preferred polydimethylsiloxanes to exhibit the appropriate  $\Delta\eta/\Delta T$  ratio, they must exhibit a viscosity at 25° C. that is within the range of 2 to 200 centipoise, preferably 5 to 100 centipoise, with 10 to 50 centipoise being especially preferred.

The fluorinated ethers and esters, class (k), of the present invention can be any linear fluorinated polymers containing a polyether or polyester backbone consisting of carbon and oxygen atoms with either  $CF_3$  or F functionality. The

preferred fluorinated ethers of the invention are perfluorinated polyethers corresponding to the following formula:



wherein A can be F or  $\text{CF}_3$  and the ratio of v:w is between about 30:1 and 50:1, preferably between about 35:1 and 45:1. Examples of commercially available perfluorinated polyethers include both the GALDEN and FOMBLIN fluorinated liquids available from Montedison USA, Incorporated.

The glycol esters and ethers, class (j), of the present invention can be any propylene or ethylene glycol derivative containing the basic structure:



wherein A is H or  $\text{CH}_3$ ; B is  $\text{CH}_3$ , H, OH, or  $\text{O}_2\text{CR}$  with R being an alkyl or aryl group; and B' is H,  $\text{CH}_3$  or  $\text{C}(\text{O})\text{R}'$  with R' being an alkyl or aryl group. The basic repeating unit as described by x may range from about 1 to 8, preferably about 1 to 4. Examples of commercially available glycol esters and ethers include the DOWANOL liquids from Dow Chemical Co.; the BENZOFLEX liquids available from Velsicol Chemical Corporation; the ARCSOLV liquids from ARCO Chemical Co.; the EKTASOLVE liquids from Eastman Kodak Co.; POLY-SOLV liquids from Olin Chemical Corporation; and the UCON, PROPASOL, CARBITOL and CELLOSOLVE liquids available from Union Carbide Corporation.

The unsaturated hydrocarbons, class (h), of the present invention can be any straight chain, branched or cyclic hydrocarbon which contains one or more carbon-carbon double or triple bonds. The unsaturated cyclic hydrocarbons appropriate to the present invention may or may not exhibit aromaticity. Examples of unsaturated hydrocarbons useful in the present invention include octene, nonene, decene, decadiene, butyl benzene, amyl benzene and toluene.

The unsaturated hydrocarbons of the present invention differ from the saturated hydrocarbons classified in classes (b) mineral oil and (g) synthetic cycloparaffins and synthetic paraffins. Saturated hydrocarbons are typically defined as straight chain, branched or cyclic hydrocarbons having all carbon-carbon single bonds. More specifically, saturated straight chain or branched hydrocarbons are termed paraffins, while saturated cyclic hydrocarbons are defined as cycloparaffins. Mineral oils, which are also known as white oils, are a mixture of paraffins and cycloparaffins obtained as a distillate of petroleum. Synthetic paraffins, which are also known as poly(olefins), are typically saturated hydrocarbons prepared through the controlled polymerization of ethylene and propylene. By definition, mineral oils is a subset of the larger class of paraffins. However, a difference in lubricating behavior demands that these two classes be differentiated, i.e., classes (b) and (g), in the present invention.

The main differentiating feature between the lubricating oil classes (b) mineral oils and (g) synthetic cycloparaffins and synthetic paraffins is that mineral oils usually exhibit higher molecular weight than their synthetic counterparts. Therefore, mineral oils typically exhibit excellent lubrication properties but have inappropriate  $\Delta\eta/\Delta T$  ratios. On the other hand, the  $\Delta\eta/\Delta T$  ratio exhibited by most oils classified in class (g) as synthetic cycloparaffins or synthetic paraffins

are usually within an acceptable range, but these class (g) fluids exhibit unacceptable lubricating properties and therefore cannot be adequately used in the present invention. Unsaturated hydrocarbons classified in class (h), on the other hand, are well known to those skilled in the art of tribology to provide better wear protection than saturated hydrocarbons of comparable viscosity and therefore can be utilized in the present invention, provided they exhibit an appropriate  $\Delta\eta/\Delta T$  ratio. Specific carrier fluids that are correctly classified in class (g) as synthetic cycloparaffins or synthetic paraffins include kerosene, mineral spirits and CONOCO LVT200 oil.

The carrier fluids appropriate to the present invention may be prepared by methods well known in the art and many are commercially available as described above. The viscosity of commercially available carrier fluids can, if needed, be reduced by techniques well known to those skilled in the art of manufacturing such compounds. Such techniques include thermal depolymerization at high temperatures and reduced pressures, as well as both acid and base depolymerization in the presence of an appropriate endblocking agent.

The carrier fluid of the present invention is typically utilized in an amount ranging from about 50 to 95, preferably from about 60 to 85, percent by volume of the total magnetorheological material. This corresponds to about 11 to 70, preferably about 15 to 41, percent by weight when the carrier fluid and particle of the magnetorheological material have a specific gravity of about 0.95 and 7.86, respectively.

It is imperative that the carrier fluids of the invention have a  $\Delta\eta/\Delta T$  ratio less than or equal to about 16.0 centipoise/ $^{\circ}\text{C}$ . over the temperature range of about  $25^{\circ}\text{C}$ . to  $-40^{\circ}\text{C}$ ., since carrier fluids having a  $\Delta\eta/\Delta T$  ratio within this range have been found to impart unexpectedly superior temperature stability to a corresponding magnetorheological material. Specifically, the low viscosity magnetorheological materials of the present invention are capable of exhibiting significantly less variance in mechanical properties over a temperature range of about  $-40^{\circ}\text{C}$ . to  $150^{\circ}\text{C}$ . than magnetorheological materials prepared with conventional carrier components. Therefore, devices (i.e., dampers, mounts, clutches, etc.) that utilize the magnetorheological materials of the invention exhibit a more constant force output over a broad temperature range than devices utilizing magnetorheological materials prepared with traditional carrier components.

The minimal variation in mechanical properties with respect to a change in temperature of the present magnetorheological materials is advantageous in that it allows for the design of smaller, more efficient devices in most applications. In addition, the magnetorheological materials of the invention allow a design engineer greater leeway in the ultimate geometry or shape of a device, as well as in methods to control the power consumption of a device. Finally, the lubricating nature of the carrier fluids of the present invention allows for improved life-time of the device by minimizing wear on individual components, such as dynamic or static seals.

The particle component of the magnetorheological material of the invention can be comprised of essentially any solid which is known to exhibit magnetorheological activity. Typical particle components useful in the present invention are comprised of, for example, paramagnetic, superparamagnetic or ferromagnetic compounds. Specific examples of particle components useful in the present invention include particles comprised of materials such as iron, iron alloys, iron oxide, iron nitride, iron carbide, carbonyl iron, chromium dioxide, low carbon steel, silicon steel, nickel, cobalt,

and mixtures thereof. The iron oxide includes all known pure iron oxides, such as  $Fe_2O_3$  and  $Fe_3O_4$ , as well as those containing small amounts of other elements, such as manganese, zinc or barium. Specific examples of iron oxides include ferrites and magnetites. In addition, the particle component can be comprised of any of the known alloys of iron, such as those containing aluminum, silicon, cobalt, nickel, vanadium, molybdenum, chromium, tungsten, manganese and/or copper. Preferred iron alloys of the invention include iron-cobalt and iron-nickel alloys. The iron-cobalt alloys preferred for use in a magnetorheological fluid have an iron:cobalt ratio ranging from about 30:70 to 95:5, preferably ranging from about 50:50 to 85:15, while the iron-nickel alloys have an iron:nickel ratio ranging from about 90:10 to 99:1, preferably ranging from about 94:6 to 97:3. The iron alloys may contain a small amount of other elements, such as vanadium, chromium, etc, in order to improve the ductility and mechanical properties of the alloys. These other elements are typically present in an amount that is less than about 3.0% by weight. Examples of iron-cobalt alloys include HYPERCO (Carpenter Technology), HYPERM (F. Krupp Widiafabrik), SUPERMENDUR (Arnold Eng.) and 2V-PERMENDUR (Western Electric).

The particle component is typically in the form of a metal powder which can be prepared by processes well known to those skilled in the art. Typical methods for the preparation of metal powders include the reduction of metal oxides, grinding or attrition, electrolytic deposition, metal carbonyl decomposition, rapid solidification, or smelt processing. Various metal powders that are commercially available include straight iron powders, reduced iron powders, insulated reduced iron powders, cobalt powders, and various alloy powders, such as [48%]Fe/[50%]Co/[2%]V. The diameter of the particles utilized herein can range from about 0.1 to 500  $\mu m$ , preferably from about 1.0 to 250  $\mu m$ , with from about 1.0 to 50  $\mu m$  being specifically preferred.

The particles may be encapsulated or covered by a surface barrier coating in order to prevent the growth of a contaminant layer that may degrade the magnetic properties of the particles. This barrier coating, which preferably encapsulates the entire particle, may be composed of a variety of materials including nonmagnetic metals, ceramics, thermoplastic polymeric materials, thermosetting polymers and combinations thereof. Examples of thermosetting polymers useful for forming a protective coating include polyesters, polyimides, phenolics, epoxies, urethanes, rubbers and silicones, while examples of thermoplastic polymeric materials include acrylics, celluloses, polyphenylene sulfides, polyquinoxilines, polyetherimides and polybenzimidazoles. Typical nonmagnetic metals useful for forming a protective coating include refractory transition metals, such as titanium, zirconium, hafnium, vanadium, niobium, tantalum, chromium, molybdenum, tungsten, copper, silver, gold, and lead, tin, zinc, cadmium, cobalt-based intermetallic alloys, and nickel-based intermetallic alloys. Examples of ceramic materials useful for forming a protective coating include the carbides, nitrides, borides, and silicides of the refractory transition metals described above; nonmetallic oxides, such as  $Al_2O_3$ ,  $Cr_2O_3$ ,  $ZrO_3$ ,  $HfO_2$ ,  $TiO_2$ ,  $SiO_2$ ,  $BeO$ ,  $MgO$ , and  $ThO_2$ ; nonmetallic nonoxides, such as  $B_4C$ ,  $SiC$ ,  $BN$ ,  $Si_3N_4$ ,  $AlN$ , and diamond; and various cermets. The preferred particles of the present invention are straight iron powders, reduced iron powders, iron-cobalt alloys and iron-nickel alloys either with or without a surface barrier coating.

The particle component typically comprises from about 5 to 50, preferably about 15 to 40, percent by volume of the total magnetorheological material depending on the desired

magnetic activity and viscosity of the overall material. This corresponds to about 30 to 89, preferably about 59 to 85, percent by weight when the carrier fluid and particle of the magnetorheological material have a specific gravity of about 0.95 and 7.86, respectively.

A surfactant to more adequately disperse the particle component in the carrier vehicle may also be optionally utilized in the magnetorheological fluid. Such surfactants include known surfactants or dispersing agents such as ferrous oleate and naphthenate, metallic soaps (e.g., aluminum tristearate and distearate), alkaline soaps (e.g., lithium and sodium stearate), sulfonates, phosphate esters, stearic acid, glycerol monooleate, sorbitan sesquioleate, stearates, laurates, fatty acids, fatty alcohols, and other surface active agents. In addition, the optional surfactant may be comprised of steric stabilizing molecules, including fluorinated polymeric esters and titanate, aluminate or zirconate coupling agents. The optional surfactant may be employed in an amount ranging from about 0.1 to 20 percent by weight relative to the weight of the particle component.

Particle settling may be minimized in the magnetorheological materials of the present invention by forming a thixotropic network. A thixotropic network is defined as a suspension of particles that, at low shear rates, form a loose network or structure sometimes referred to as clusters or flocculates. The presence of this three-dimensional structure imparts a small degree of rigidity to the magnetorheological material, thereby reducing particle settling. However, when a shearing force is applied through mild agitation, this structure is easily disrupted or dispersed. When the shearing force is removed, this loose network is reformed over a period of time. A thixotropic network may be formed in the magnetorheological fluid of the present invention through the utilization of any known thixotropic additive such as hydrogen-bonding thixotropic agents and/or colloidal additives. The thixotropic agents and colloidal additives, if utilized, are typically employed in an amount ranging from about 0.1 to 5.0, preferably from about 0.5 to 3.0, percent by volume relative to the overall volume of the magnetorheological fluid.

Examples of hydrogen-bonding thixotropic agents useful in the present invention include low molecular weight hydrogen-bonding molecules containing hydroxyl, carboxyl or amine functionality, as well as medium molecular weight hydrogen-bonding molecules, such as silicone oligomers, organosilicone oligomers, and organic oligomers. Typical low molecular weight hydrogen-bonding molecules include alcohols; glycols; alkyl amines, amino alcohols, amino esters, and mixtures thereof. Typical medium molecular weight hydrogen-bonding molecules include oligomers containing sulphonated, amino, hydroxyl, cyano, halogenated, ester, carboxylic acid, ether, and ketone moieties, as well as mixtures thereof.

Examples of colloidal additives useful in the present invention include hydrophobic and hydrophilic metal oxide and high molecular weight powders. Examples of hydrophobic powders include surface-treated hydrophobic fumed silica and organo-clays. Examples of hydrophilic metal oxide or polymeric materials include silica gel, fumed silica, clays, and high molecular weight derivatives of castor oil, poly(ethyleneoxide), and poly(ethylene glycol).

The magnetorheological fluid of the invention may also contain other optional additives such as dyes or pigments, abrasive particles, lubricants, pH shifters, salts, deacidifiers, or corrosion inhibitors. These optional additives may be in the form of dispersions, suspensions, or materials that are soluble in the carrier vehicle.

The magnetorheological materials of the present invention can be prepared by initially mixing the ingredients together by hand (low shear) with a spatula or the like and then subsequently more thoroughly mixing (high shear) with a homogenizer, mechanical mixer or shaker or dispersing with an appropriate milling device such as a ball mill, sand mill, attritor mill, paint mill, colloid mill or the like, in order to create a more stable suspension.

Evaluation of the mechanical properties and characteristics of the magnetorheological materials of the present invention, as well as other magnetorheological materials, can be obtained through the use of parallel plate and/or concentric cylinder couette rheometry. The theories which provide the basis for these techniques are further described by S. Oka in *Rheology, Theory and Applications* (volume 3, F. R. Eirich, ed., Academic Press: New York, 1960). The information that can be obtained from a rheometer includes data relating mechanical shear stress as a function of shear strain rate. For magnetorheological materials, the shear stress versus shear strain rate data can be modeled after a Bingham plastic in order to determine the dynamic yield stress and viscosity. Within the confines of this model the dynamic yield stress for the magnetorheological material corresponds to the zero-rate intercept of a linear regression curve fit to the measured data. The viscosity of the material is defined as the slope of the line generated by this curve fitting technique. The magnetorheological effect at a particular magnetic field can be further defined as the difference between the dynamic yield stress measured at that magnetic field and the dynamic yield stress measured when no magnetic field is present.

In a concentric cylinder cell configuration the magnetorheological material is placed in the annular gap formed between an inner cylinder of radius  $R_1$  and an outer cylinder of radius  $R_2$ , while in a simple parallel plate configuration the material is placed in the planar gap formed between upper and lower plates both with a radius,  $R_3$ . In these techniques either one of the plates or cylinders is then rotated with an angular velocity  $\omega$  while the other plate or cylinder is held motionless. A magnetic field is typically applied to these cell configurations across the fluid-filled gap, either radially for the concentric cylinder configuration, or axially for the parallel plate configuration. The relationship between the shear stress and the shear strain rate is then derived from this angular velocity and the torque,  $T$ , applied to maintain or resist it.

The testing of various application specific devices, such as dampers, mounts and clutches, that utilize either the magnetorheological materials of the present invention or other magnetorheological materials, is a second method of evaluating the mechanical performance of these materials. The magnetorheological material-containing device is simply placed in line with a mechanical actuator and operated with a specified displacement amplitude and frequency. A magnetic field is appropriately applied to the device and the force output determined from the resulting extension/compression waveforms plotted as a function of time. The methodology utilized to test dampers, mounts and clutches is well known to those skilled in the art of vibration control.

The following examples are given to illustrate the invention and should not be construed to limit the scope of the invention. In the examples, all viscosities are stated as being measured at a specific temperature and are given in centipoise.

#### EXAMPLES 1-9

The  $\Delta\eta/\Delta T$  ratio for various Group I carrier fluids selected from the groups (h) through (n) are measured using con-

ventional rheometry techniques in conjunction with a concentric cylinder or couette cell. The temperature of the carrier fluid is measured using a thermocouple in contact with the fluid through out the entire test. The  $\Delta\eta/\Delta T$  ratio is defined as the viscosity measured for the carrier fluid at  $-40^\circ C$ . minus the viscosity of the carrier fluid measured at  $25^\circ C$ ., the sum of which is divided by  $65^\circ C$ . to yield a ratio given in units of centipoise/ $^\circ C$ . The variance in the measurements obtained by this method is found by repetitive testing of several fluids to be about  $\pm 0.5$  mPa-sec/ $^\circ C$ . The  $\Delta\eta/\Delta T$  ratios measured for carrier fluids appropriate to the present invention are summarized in Table 1.

TABLE 1

| Example # | Group Classification        | Carrier Fluid Description                                                                             | $\Delta\eta/\Delta T$ ratio |
|-----------|-----------------------------|-------------------------------------------------------------------------------------------------------|-----------------------------|
| 1         | (i) mono-basic acid ester   | propyl benzoate (#30,700-9, Aldrich Chemical Co.)                                                     | 5.5                         |
| 2         | (j) glycol ester/ether      | dipropylene glycol n-butyl ether (DOWANOL DPnB, Dow Chemical Company)                                 | 3.5                         |
| 3         | (j) glycol ester/ether      | propylene glycol n-butyl ether (DOWANOL PnB, Dow Chemical Company)                                    | 0.9                         |
| 4         | (j) glycol ester/ether      | copolymer of ethylene & propylene oxide (UCON 50-HB-55, Union Carbide Chemicals & Plastics Co., Inc.) | 15.9                        |
| 5         | (k) fluorinated ester/ether | fluorinated polyether (GALDEN D02, Montedison USA, Inc.)                                              | 0.5                         |
| 6         | (k) fluorinated ester/ether | fluorinated polyether (GALDEN D10, Montedison USA, Inc.)                                              | 11.2                        |
| 7         | (m) silicone oil            | polydimethylsiloxane (L-45, 10 cstk, Union Carbide Chemicals & Plastics Co., Inc.)                    | 0.6                         |
| 8         | (m) silicone oil            | polydimethylsiloxane (PS040, 50 cstk, Huls America Inc.)                                              | 3.6                         |
| 9         | (m) silicone oil            | polydimethylsiloxane (L-45, 200 cstk, Union Carbide Chemicals & Plastics Co., Inc.)                   | 13.9                        |

Examples 1-9 demonstrate that certain fluids within the main lubricating oils classes or groups (h) through (n) exhibit a  $\Delta\eta/\Delta T$  ratio less than about 16 centipoise/ $^\circ C$ . with preferred Group I fluids exhibiting a ratio less than about 9 centipoise/ $^\circ C$ . and especially preferred Group I fluids having a ratio less than about 7 centipoise/ $^\circ C$ . Examples 7-9 further establish the viscosity limit for polydimethylsiloxanes to be about 200 cstk in order to exhibit the necessary  $\Delta\eta/\Delta T$  ratio.

#### COMPARATIVE EXAMPLES 10-22

The  $\Delta\eta/\Delta T$  ratio for various Group II carrier fluids selected from within the lubricating oil groups (h through n) are measured using the procedure described for Examples 1-9. The  $\Delta\eta/\Delta T$  ratios measured for these comparative carrier fluids are summarized in Table 2.

TABLE 2

| Example # | Group Classification      | Carrier Fluid Description                                    | $\Delta\eta/\Delta T$ ratio |
|-----------|---------------------------|--------------------------------------------------------------|-----------------------------|
| 10        | (i) mono-basic acid ester | butyl benzoate (#29,329-6, Aldrich Chemical Co.)             | *Thick                      |
| 11        | (j) glycol ester/ether    | ethylene glycol phenyl ether (DOWANOL EPH, Dow Chemical Co.) | *Thick                      |
| 12        | (j) glycol                | propylene glycol (#13,436-8,                                 | 438.0                       |

TABLE 2-continued

| Example # | Group Classification         | Carrier Fluid Description                                                                                                      | $\Delta\eta/\Delta T$ ratio |
|-----------|------------------------------|--------------------------------------------------------------------------------------------------------------------------------|-----------------------------|
| 13        | (j) glycol ester/ether       | Aldrich Chemical Co.) copolymer of propylene & ethylene oxide (UCON LB-65, Union Carbide Chemical & Plastics Co., Inc.)        | 57.0                        |
| 14        | (j) glycol ester/ether       | copolymer of propylene & ethylene oxide (UCON 50-HB-100, Union Carbide Chemical & Plastics Co., Inc.)                          | 111.0                       |
| 15        | (j) glycol ester/ether       | copolymer of propylene & ethylene oxide (UCON LB-135, Union Carbide Chemical & Plastics Co., Inc.)                             | 437.0                       |
| 16        | (k) fluorinated ether/ether  | fluorinated polyether (GALDEN D20, Montedison USA, Inc.)                                                                       | 60.0                        |
| 17        | (k) fluorinated ether/ether  | perfluorinated polyether (FOMBLIN L-VAC 25/6, Montedison USA, Inc.)                                                            | 483.0                       |
| 18        | (l) silicate ester           | tetraphenylsilicate (T2075, mp = 48° C., tetraphenoxy-silane, Huls America Inc.)                                               | **solid at low T            |
| 19        | (m) silicone oil             | polydimethylsiloxane (PS041.5, 350 cstk, Huls America Inc.)                                                                    | 34.2                        |
| 20        | (m) silicone oil             | polymethylphenylsiloxane (PS160, 500 cstk, Huls America Inc.)                                                                  | *Thick                      |
| 21        | (m) silicone oil             | poly(methyl-3,3,3-trifluoropropyl) siloxane (FS1265, 300 cstk, Dow Corning Corp.)                                              | *Thick                      |
| 22        | (n) halogenated hydrocarbons | chlorinated biphenyls: i.e., 4-chloro biphenyl (mp = 78° C.), 2-chloro biphenyl (mp = 34° C.), 3-chloro biphenyl (mp = 16° C.) | ***solid at low T           |

\*Fluid became too thick to test, thus  $\Delta\eta/\Delta T$  ratio >> 16

\*\*data obtained from Huls America Inc.

\*\*\*data obtained from CRC, 67th ed., 1986, page C-154

Examples 10–22 demonstrate that a considerable number of carrier fluids exist within the lubricating oil groups (h) through (n) that do not exhibit the necessary  $\Delta\eta/\Delta T$  ratio for utilization as part of the present invention. A device utilizing a magnetorheological material containing these comparative carrier fluids will exhibit a large variation in force output when operated over a broad temperature range. Examples 18 and 22 demonstrate that specific carrier fluids, such as tetraphenylsilicate ester and chlorinated biphenyls of U.S. Pat. No. 2,751,352 that do not satisfy the necessary  $\Delta\eta/\Delta T$  ratio as described by the present invention. Example 19 demonstrates that a polydimethylsiloxane whose viscosity is greater than the limit of 200 cstk as previously described in Example 9 exhibits an unsatisfactory  $\Delta\eta/\Delta T$  ratio.

## COMPARATIVE EXAMPLES 23–33

The  $\Delta\eta/\Delta T$  ratio for various Group II carrier fluids selected from within the lubricating oil groups (a) through (e) are measured using the procedure described for Examples 1–9. The  $\Delta\eta/\Delta T$  ratios measured for these comparative carrier fluids are summarized in Table 3.

TABLE 3

| Example # | Group Classification   | Carrier Fluid Description                                                        | $\Delta\eta/\Delta T$ ratio |
|-----------|------------------------|----------------------------------------------------------------------------------|-----------------------------|
| 5         | (d) dibasic acid ester | di(2-ethylhexyl) sebacate (#29,083-1 Aldrich Chemical Co.)                       | 26.0                        |
| 23        | (d) dibasic acid ester | di(2-ethylhexyl) adipate (KODAFLEX DOA plasticizer, Eastman Chemical Co.)        | 27.0                        |
| 24        | (d) dibasic acid ester | di(octyl) phthalate (#D20,115-4, Aldrich Chemical Co.)                           | 43.0                        |
| 25        | (d) dibasic acid ester | dibutyl sebacate (#24,047-8, Aldrich Chemical Co.)                               | *Thick                      |
| 26        | (d) dibasic acid ester | ethylRicinoleate (TCI, Japan)                                                    | *Thick                      |
| 27        | (d) dibasic acid ester | white mineral oil (DRAKEOL 10B, 18 cstk, Penreco, Div. of Pennzoil Products Co.) | 179.0                       |
| 28        | (b) mineral oils       | hydraulic oil (MOBIL DTE-13M, 33 cstk, Mobil Oil Corp.)                          | 41.0                        |
| 29        | (b) mineral oils       | hydraulic oil (MOBIL DTE-11, 15 cstk, Mobil Oil Corp.)                           | 83.7                        |
| 30        | (b) mineral oils       | white, light mineral oil (#33,077-9, Aldrich Chemical Co.)                       | 38.9                        |
| 31        | (b) mineral oils       | white mineral oil (DRAKEOL 5, 8 cstk, Penreco, Div. of Pennzoil Products Co.)    | *Thick                      |
| 32        | (b) mineral oils       | mineral oil (#6081, Viscosity Oil Inc.)                                          | 196.0                       |

\*Fluid became too thick to test, thus  $\Delta\eta/\Delta T$  ratio >> 16

Examples 23–33 demonstrate that carrier fluids selected from the lubricating oil groups (a) through (e) do not exhibit the necessary  $\Delta\eta/\Delta T$  ratio to minimize force output of a magnetorheological material device when operated over a broad temperature range. These examples also demonstrate that most conventional carrier components in the lubricating oil groups (a) through (e) that have been previously described in the literature (e.g., U.S. Pat. No. 2,751,352)

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715

TABLE 4

| Example # | Group Classification    | Carrier Fluid Description                                                                                                                                                                                                                  | $\Delta\eta/\Delta T$ ratio |
|-----------|-------------------------|--------------------------------------------------------------------------------------------------------------------------------------------------------------------------------------------------------------------------------------------|-----------------------------|
| 34        | primary fluid mixture   | 25% GALDEN D02 (group k, $\Delta\eta/\Delta T = 0.5$ , Example 5) and 75% GALDEN D20 (group k, $\Delta\eta/\Delta T = 60.0$ , Example 16)                                                                                                  | 7.0                         |
| 35        | primary fluid mixture   | 50% GALDEN D02 and 50% GALDEN D20                                                                                                                                                                                                          | 4.1                         |
| 36        | primary fluid mixture   | 75% GALDEN D02 and 25% GALDEN D20                                                                                                                                                                                                          | 0.6                         |
| 37        | secondary fluid mixture | 25% CONOCO LVT-200 (mixture of synthetic paraffins and cyclopolyaraffins, group g, $\Delta\eta/\Delta T = 0.5$ , Conoco Inc.) and 75% di(2-ethylhexyl) sebacate (group d, $\Delta\eta/\Delta T = 26.0$ , Example 29)                       | 8.6                         |
| 38        | secondary fluid mixture | 50% CONOCO LVT-200 and 50% di(2-ethylhexyl) sebacate                                                                                                                                                                                       | 2.7                         |
| 39        | secondary fluid mixture | 75% CONOCO LVT-200 and 25% di(2-ethylhexyl) sebacate                                                                                                                                                                                       | 1.5                         |
| 40        | secondary fluid mixture | Mixture of 50% #6098 oil (polyolefin or synthetic paraffin, group g, $\Delta\eta/\Delta T = 12.0$ , Viscosity Oil Inc.) and 50% #6081 oil (group b, $\Delta\eta/\Delta T = 196.0$ , Example 28) supplied as #6097 oil (Viscosity Oil Inc.) | 6.7                         |

Examples 34–36 demonstrate that primary fluid mixtures that exhibit acceptable  $\Delta\eta/\Delta T$  ratios can be obtained by mixing a carrier fluid selected from the Group I carrier fluids with a carrier fluid selected from the Group II carrier fluids. Between 25 and 75% by weight of a Group I carrier fluid is needed to insure that the primary fluid mixture exhibits acceptable lubricating properties. Examples 37–40 demonstrate that secondary fluid mixtures that exhibit acceptable  $\Delta\eta/\Delta T$  ratios can be obtained by mixing a carrier fluid selected from the Group III carrier fluids with a carrier fluid selected from the Group IV carrier fluids. Between 25 to 75% by weight of a carrier fluid selected from the Group III carrier fluids is needed to insure that the secondary fluid mixture exhibits an acceptable  $\Delta\eta/\eta T$  ratio. However, a minimum of 25% by weight of the carrier fluid selected from the Group IV carrier fluids is necessary to insure that the secondary fluid mixture exhibits acceptable lubricating properties.

Example 40 demonstrates that the secondary fluid mixture can unexpectedly exhibit a  $\Delta\eta/\Delta T$  ratio that is smaller than the  $\Delta\eta/\Delta T$  ratios measured for the individual fluids that are used to prepare the mixture. One would normally expect that the  $\Delta\eta/\Delta T$  ratio of a fluid mixture would fall between the  $\Delta\eta/\Delta T$  ratios exhibited by the individual fluids that make up the mixture. This result allows for some secondary fluid mixtures to exhibit improved lubricating properties by being able to incorporate a larger amount of the carrier fluids selected from the Group IV carrier fluids into the mixture without adversely affecting the  $\Delta\eta/\Delta T$  ratio exhibited by the mixture.

#### COMPARATIVE EXAMPLES 41–43

The  $\Delta\eta/\Delta T$  ratio for various carrier fluid mixtures wherein the carrier fluids are selected from within the fluid classes (a) through (n) are measured using the procedure described for Examples 1–9. The  $\Delta\eta/\Delta T$  ratios measured for these comparative carrier fluids are summarized in Table 5.

TABLE 5

| Example # | Group Classification      | Carrier Fluid Description                                                                                                               | $\Delta\eta/\Delta T$ ratio |
|-----------|---------------------------|-----------------------------------------------------------------------------------------------------------------------------------------|-----------------------------|
| 41        | Comparative fluid mixture | 25% DRAKEOL 5 ( $\Delta\eta/\Delta T > 16$ , Example 27) and 75% di(2-ethylhexyl) sebacate ( $\Delta\eta/\Delta T = 26.0$ , Example 29) | 47.0                        |
| 42        | Comparative fluid mixture | 50% DRAKEOL 5 and 50% di(2-ethylhexyl) sebacate                                                                                         | 46.2                        |
| 43        | Comparative fluid mixture | 75% DRAKEOL 5 and 25% di(2-ethylhexyl) sebacate                                                                                         | 47.3                        |

Examples 41–43 demonstrate that if individual carrier fluids are not properly selected as previously defined for primary and secondary fluid mixtures the resulting carrier fluid mixture will not exhibit an appropriate  $\Delta\eta/\Delta T$  ratio.

#### EXAMPLE 44

A magnetorheological material is prepared by adding together a total of 1257.6 g straight carbonyl iron powder (MICROPOWDER-S1640, which is similar to old E1 iron powder notation, from GAF Chemicals Corporation), 25.0 g Mn/Zn ferrite (#73302-0, D. M. Steward Manufacturing Company), 17.3 g siloxane oligomer-modified silica (CABOSIL TS720, Cabot Corporation) as a polymer-modified metal oxide, and 25.2 g of a phosphate ester dispersant (EMPHOS CS141, Witco Chemical Corporation) with 294.7 g polydimethylsiloxane oil (Example 7). The viscosity of the polydimethylsiloxane selected from group (m) is measured by concentric cylinder rheometry to be about 16 centipoise at 25° C. The magnetorheological material is made into a homogeneous mixture over a 16-hour period using an attritor mill. The material is stored in a polyethylene container until utilized.

#### COMPARATIVE EXAMPLE 45

A magnetorheological material is prepared according to the procedure described in Example 44. However, in this example the 16 centipoise polydimethylsiloxane oil is replaced with a higher viscosity silicone oil (PS042, 500 centistoke, Huls America Inc.). The viscosity of this silicone oil selected from group (m) is measured by concentric cylinder rheometry to be about 660 centipoise at 25° C. The magnetorheological material is stored in a polyethylene container until utilized.

#### Mechanical Properties of Examples 44 and 45

The mechanical performance of the magnetorheological materials prepared in Examples 44 and 45 are evaluated in a linear magnetorheological damper over a temperature range of -40° to 150° C. More specifically, this damper contains approximately 250 mL of a magnetorheological material that is forced to flow by the movement of a piston. A magnetic field is generated and controlled across a gap within the device through the application of electric current to an electromagnetic coil contained within the piston. The width of this gap through which the fluid flows is about 1.5 mm. During the tests the damper is operated at a frequency of 1.0 Hz with a displacement amplitude of  $\pm 0.5$  inch. A magnetic field is appropriately applied to the device and the force output determined from the resulting extension/compression waveforms plotted as a function of time.

The force output of this linear damper utilizing a low viscosity magnetorheological material of the present invention (Example 44) is compared in FIG. 1 to the force output of this same damper using a high viscosity comparative magnetorheological material (Example 45). In this figure the measured force data at a magnetic field of about 1000 Oersted is plotted as a function of temperature. The damper utilizing a magnetorheological material of the invention is observed to provide a relatively constant (less than about 15% variation) force output over the temperature range of -40° to 150° C., while the force output of this same damper varies by greater than about 70% over this temperature range when the comparative magnetorheological material of Example 45 is utilized.

#### EXAMPLE 46

A magnetorheological material is prepared by adding together a total of 235.80 g straight carbonyl iron powder (MICROPOWDER-S-1640, GAF Chemicals Corporation) and 6.90 g siloxane oligomer-modified silica (CABOSIL TS 720, Cabot Corporation) as a thixotrope with 56.01 g secondary fluid mixture (#6097 oil, Example ). The weight amount of iron particles in this magnetorheological material corresponds to a volume fraction of 0.30. The secondary fluid mixture exhibits a  $\Delta\eta/\Delta T$  ratio of 6.7 centipoise/°C. over the temperature range of 25° C. to -40° C. The magnetorheological material is made into a homogeneous mixture through the use of a high speed mechanical disperser. The material is stored in a polyethylene container until utilized.

#### EXAMPLE 47

A magnetorheological material is prepared according to the procedure described in Example 46. However, in this example 235.80 g straight carbonyl iron powder (MICROPOWDER-S-1640, GAF Chemicals Corporation) is added to 129.50 g perfluorinated polyether (Galder D 10, Montedison USA, Inc.). The weight amount of iron particles in this magnetorheological material corresponds to a volume fraction of 0.30. The carrier fluid selected from group (k) has a  $\Delta\eta/\Delta T$  ratio of 11.2 centipoise/°C. over the temperature range of 25° C. to -40° C. The magnetorheological material is stored in a polyethylene container until utilized.

#### EXAMPLE 48

A magnetorheological material is prepared according to the procedure described in Example 46. However, in this example 235.80 g straight carbonyl iron powder (MICROPOWDER-S-1640, GAF Chemicals Corporation) is added to 71.82 g propyl benzoate (#30,700-9, Aldrich Chemical Company). The weight amount of iron particles in this magnetorheological material corresponds to a volume fraction of 0.30. The carrier fluid selected from group (i) has a  $\Delta\eta/\Delta T$  ratio of 5.5 centipoise/°C. over the temperature range of 25° C. to -40° C. The magnetorheological material is stored in a polyethylene container until utilized.

#### COMPARATIVE EXAMPLE 49

A magnetorheological material is prepared according to the procedure described in Example 46. However, in this example 235.80 g straight carbonyl iron powder (MICROPOWDER-S-1640, GAF Chemicals Corporation) and 6.90 g siloxane oligomer-modified silica (CABOSIL TS-720, Cabot Corporation) as a thixotrope are added to 56.08 g white mineral oil (Example 27). The weight amount

of iron particles in this magnetorheological material corresponds to a volume fraction of 0.30. The carrier fluid selected from group (b) has a  $\Delta\eta/\Delta T$  ratio that is significantly greater than 16.0 centipoise/°C. over the temperature range of 25° C. to -40° C. The magnetorheological material is stored in a polyethylene container until utilized.

#### COMPARATIVE EXAMPLE 50

A magnetorheological material is prepared according to the procedure described in Example 46. However, in this example 235.80 g straight carbonyl iron powder (MICROPOWDER-S-1640, GAF Chemicals Corporation) is added to 133.00 g perfluorinated polyether (Example 17). The weight amount of iron particles in this magnetorheological material corresponds to a volume fraction of 0.30. The carrier fluid selected from group (k) has a  $\Delta\eta/\Delta T$  ratio of 483.0 centipoise/°C. over the temperature range of 25° C. to -40° C. The magnetorheological material is stored in a polyethylene container until utilized.

#### COMPARATIVE EXAMPLE 51

A magnetorheological material is prepared according to the procedure described in Example 46. However, in this example 235.80 g straight carbonyl iron powder (MICROPOWDER-S-1640, GAF Chemicals Corporation) is added to 70.70 g butyl benzoate (Example 10). The weight amount of iron particles in this magnetorheological material corresponds to a volume fraction of 0.30. The carrier fluid selected from group (i) has a  $\Delta\eta/\Delta T$  ratio that is significantly greater than 16.0 centipoise/°C. over the temperature range of 25° C. to -40° C. The magnetorheological material is stored in a polyethylene container until utilized.

#### Mechanical Properties of Examples 46 and 49

The mechanical performance of the magnetorheological materials prepared in Example 46 and comparative Example 49 are evaluated in a linear magnetorheological damper over a temperature range of -40° to 50° C. More specifically, this damper contains approximately 50 mL of a magnetorheological material that is forced to flow by the movement of a piston. A magnetic field is generated and controlled across a gap within the device through the application of electric current to an electromagnetic coil contained within the piston. The width of this gap through which the fluid flows is about 1.5 mm. During the tests the damper is operated at a frequency of 1.0 Hz with a displacement amplitude of  $\pm 0.5$  inch. A magnetic field is appropriately applied to the device and the force output determined from the resulting extension/compression waveforms plotted as a function of time.

The force output of the linear damper utilizing the low viscosity magnetorheological material of the present invention (Example 46) is compared in FIG. 2 to the force output of this same damper using a comparative magnetorheological material (Example 49). In this figure the measured force data at a magnetic field of about 1000 Oersted is plotted as a function of temperature. The damper utilizing the magnetorheological material of the invention is observed to provide a relatively constant (less than about 34% variation) force output over the temperature range of -40° to 150° C., while the force output of this same damper varies by greater than about 69% over this temperature range when the comparative magnetorheological material of Example 49 is utilized. In fact, when the comparative magnetorheological material (Example 49) is utilized, the maximum force limit

(safe operating limit) of the damper is exceeded at low temperatures.

#### Mechanical Properties of Examples 47 and 50

The mechanical properties of Examples 47 and 50 are evaluated by the procedure previously described for Examples 46 and 49. The force output of the linear damper utilizing the low viscosity magnetorheological material of the present invention (Example 47) is compared in FIG. 3 to the force output of this same damper using a comparative magnetorheological material (Example 50). In this figure the measured force data at a magnetic field of about 1000 Oersted is plotted as a function of temperature. The damper utilizing the magnetorheological material of the invention is observed to provide a relatively constant (less than about 30% variation) force output over the temperature range of -40° to 150° C., while the force output of this same damper varies by greater than about 61% over this temperature range when the comparative magnetorheological material of Example 50 is utilized. In fact, when the comparative magnetorheological material (Example 50) is utilized, the maximum force limit (safe operating limit) of the damper is exceeded at low temperatures.

#### Mechanical Properties of Examples 47 and 51

The force output of the linear damper utilizing the low viscosity magnetorheological material of the present invention (Example 47) is compared in FIG. 4 to the force output of this same damper using a comparative magnetorheological material (Example 51). In this figure the measured force data at a magnetic field of about 1000 Oersted is plotted as a function of temperature. The damper utilizing the magnetorheological material of the invention is observed to provide a relatively constant (less than about 11% variation) force output over the temperature range of -40° to 150° C., while the force output of this same damper varies by greater than about 67% over this temperature range when the comparative magnetorheological material of Example 51 is utilized. In fact, when the comparative magnetorheological material (Example 51) is utilized, the maximum force limit (safe operating limit) of the damper is exceeded at low temperatures.

#### Magnetorheological Effect Exhibited by Examples 44-51

The mechanical properties of the magnetorheological materials prepared in Examples 44-51 are further evaluated through the use of parallel plate rheometry. All the magnetorheological materials are observed to similarly exhibit significant dynamic yield stress values at 25° C. at various magnetic field strengths. For example, dynamic yield stress values of 43 and 52 kPa were measured for the magnetorheological material of Example 47 at magnetic field strengths of 2000 and 3000 Oersted, respectively. The dynamic yield stress value is defined as the y-intercept of a linear regression curve fit to the shear stress versus strain rate data obtained from the rheometer. A measure of the magnetorheological effect exhibited by a material is the difference that exists between the dynamic yield stress values observed in the presence of a magnetic field (on-state) and the yield stress value observed in the absence of a magnetic field (off-state). The off-state, dynamic yield stress values for the magnetorheological materials of Examples 44-51 are measured to be less than 1 kPa.

As can be seen from the above examples, the magnetorheological materials of the present invention exhibit significant magnetorheological activity and are capable of exhibiting stable performance over a temperature range of -40° to 150° C. The consistent performance of the present materials at the diverse temperatures described above is unexpected in light of the highly variable performance of traditional magnetorheological materials under similar diverse temperature conditions.

It is understood that the foregoing is a description of the preferred embodiments of the present invention and that the scope of the invention is not limited to the specific terms and conditions set forth above but is determined by the following claims.

What is claimed is:

1. A magnetorheological material comprising:
  - a) a carrier fluid selected from the group consisting of silicon oils and having a  $\Delta\eta/\Delta T$  ratio less than or equal to about 16 centipoise/°C. over a temperature range of about -40° to 25° C.; and,
  - b) a particle component wherein said particle component consists of particles having diameters from about 1.0 to 250 microns and having magnetorheological activity, wherein said magnetorheological material exhibits minimal variation in force output over a temperature range from about -40° C. to 150° C.
2. A magnetorheological material according to claim 1 wherein said silicone oils are selected from the group consisting of polydimethylsiloxanes, polymethylphenylsiloxanes, poly(methyl-3,3,3-trifluoropropyl)siloxanes, poly-chlorophenylmethylsiloxanes, dimethyl(tetrachlorophenyl) siloxane copolymers, dimethyl(phenylmethyl)siloxane copolymers, dimethyl(diphenyl)siloxane copolymers, and methyl-3,3,3-trifluoropropyl (dimethyl )siloxane copolymers.
3. A magnetorheological material according to claim 1 wherein the  $\Delta\eta/\Delta T$  ratio is less than or equal to about 9 centipoise/°C.
4. A magnetorheological material according to claim 3 wherein the  $\Delta\eta/\Delta T$  ratio is less than or equal to about 7 centipoise/°C.
5. A magnetorheological material according to claim 1 wherein the particle component is selected from the group consisting of iron, iron alloys, iron oxide, iron nitride, iron carbide, carbonyl iron, chromium dioxide, low carbon steel, silicon steel, nickel, cobalt, and mixtures thereof.
6. A magnetorheological material according to claim 1 wherein the particle component is covered by a surface barrier coating.
7. A magnetorheological material according to claim 6 wherein the barrier coating is composed of a material selected from the group consisting of nonmagnetic metals, ceramics, thermoplastic polymeric materials, thermosetting polymers and combinations thereof.
8. A magnetorheological material according to claim 1 further comprising a surfactant.
9. A magnetorheological material according to claim 1 further comprising a thixotropic additive selected from the group consisting of hydrogen bonding thixotropic agents and colloidal additives.
10. A magnetorheological material according to claim 1 wherein the carrier fluid is present in an amount ranging from about 50 to 95 percent by volume and the particle component is present in an amount ranging from about 5 to 50 percent by volume of the total magnetorheological material.
11. A magnetorheological material according to claim 10 wherein the carrier fluid is present in an amount from about

60 to 85 percent by volume and the particle component is present in an amount from about 15 to 40 percent by volume of the total magnetorheological material.

12. The magnetorheological material of claim 1 wherein said particle component consists of particles having diameter from about 1.0 to 50 microns.

13. A magnetorheological material according to claim 1 wherein said silicon oil has a viscosity within the range of 20 to 200 centipoise at 25° C.

14. A magnetorheological material comprising:

a) a carrier fluid selected from the group consisting of glycol esters and ethers and having a  $\Delta\eta/\Delta T$  ratio less than or equal to about 16 centipoise/°C. over a temperature range of about -40° C. to 25° C. and,

b) a particle component wherein said particle component consists of particles having diameters from about 1.0 to 250 microns and having magnetorheological activity, wherein said magnetorheological material exhibits minimal variation in force output over a temperature range from about -40° C. to 150° C.

15. A magnetorheological material according to claim 1 wherein the glycol esters and ethers are propylene or ethylene glycol derivatives containing the basic structure:



wherein A is H or  $\text{CH}_3$ ; B is  $\text{CH}_3$ , H, OH, or  $\text{O}_2\text{CR}$  with R being an alkyl or aryl group; B' is H,  $\text{CH}_3$  or  $\text{C}(\text{O})\text{R}'$  with R' being an alkyl or aryl group; and x ranges from about 1 to 8.

16. A magnetorheological material comprising:

a) a carrier fluid selected from the group consisting of monobasic acid esters and having a  $\Delta\eta/\Delta T$  ratio less than or equal to about 16 centipoise/°C. over a temperature range of about -40° to 25° C. and,

b) a particle component wherein said particle component consists of particles having diameters from about 1.0 to 250 microns and having magnetorheological activity, wherein said magnetorheological material exhibits minimal variation in force output over a temperature range from about -40° C. to 150° C.

17. A magnetorheological material comprising:

a) a carrier fluid selected from the group consisting of silicate esters and having a  $\Delta\eta/\Delta T$  ratio less than or equal to about 16 centipoise/°C. over a temperature range of about -40° to 25° C. and,

b) a particle component wherein said particle component consists of particles having diameters from about 1.0 to 250 microns and having magnetorheological activity,

45

wherein said magnetorheological material exhibits minimal variation in force output over a temperature range from about -40° C. to 150° C.

18. A magnetorheological material comprising:

a) a mixture of carrier fluids wherein the mixture of carrier fluids has a  $\Delta\eta/\Delta T$  ratio less than or equal to about 16 centipoise/°C. over a temperature range of about -40° C. to 25° C.; and,

b) a particle component wherein said particle component consists of particles having diameters from about 1.0 to 250 microns and having magnetorheological activity, wherein said magnetorheological material exhibits minimal variation in force output over a temperature range from about -40° C. to 150° C.

19. A magnetorheological material according to claim 18

wherein said mixture of carrier fluids consists of a mixture of a Group I carrier fluid selected from the group consisting of unsaturated hydrocarbon oils, glycol esters and ethers, fluorinated esters and ethers, and silicone oils and a Group

20 II carrier fluid selected from the group consisting of natural fatty oils, mineral oils, dibasic acid esters, synthetic cycloparaffins and synthetic paraffins, unsaturated hydrocarbon oils, glycol esters and ethers, fluorinated esters and ethers

25 and silicone oils, said Group II carrier fluid having a  $\Delta\eta/\Delta T$  ratio greater than about 16 centipoise/°C. over a temperature range from about -40° C. to 25° C.

20. A magnetorheological material according to claim 19 wherein the Group I and Group II carrier fluids are present in a Group I:Group II weight ratio of about 85:15.

21. A magnetorheological material according to claim 20 wherein the ratio is about 75:25.

22. A magnetorheological material according to claim 21 wherein the ratio is about 50:50.

23. A magnetorheological material according to claim 18 wherein said mixture of carrier fluids consists of a mixture of a Group III carrier fluid selected from the group consisting of synthetic cycloparaffins and synthetic paraffins and a Group IV carrier fluid selected from the group consisting of natural fatty oils, mineral oils, dibasic acid esters, unsaturated hydrocarbon oils, glycol esters and ethers, and fluorinated esters and ethers.

24. A magnetorheological material according to claim 23 wherein the Group III and Group IV carrier fluids are present in a Group III:Group IV weight ratio of about 85:15.

25. A magnetorheological material according to claim 24 wherein the ratio is about 75:25.

26. A magnetorheological material according to claim 25 wherein the ratio is about 50:50.

\* \* \* \* \*